

## UNITED STATES PATENT OFFICE

1,963,619

## EXPLOSIVE COMPOSITION

Karl T. Gent, Terre Haute, Ind., and Norman G. Johnson, Woodbury, N. J., assignors to E. I. du Pont de Nemours & Company, Wilmington, Del., a corporation of Delaware

No Drawing. Application February 23, 1932,  
Serial No. 594,734

14 Claims. (Cl. 52—11)

This invention relates to an improvement in explosive compositions having a liquid explosive ingredient as a sensitizing agent, and in particular to such a composition of the permissible dynamite type including a carbonaceous combustible material comprising certain selected parts of cereal grains.

Low density dynamites have assumed a position of particular importance in recent years. The advantages of these explosives are many in the blasting of materials having relatively low resistance such for example as coal, salt, and soft rock. Since by such means the distribution of the strength of the explosive over a considerable bore hole surface is effected, and at the same time undue shattering of the material to be blasted is in a great measure prevented. These and numerous other advantages of low density dynamite compositions of the several types are well known in the art.

Low density dynamites have heretofore been produced by a variety of means and compositions, important among which are such carbonaceous combustible ingredients as bagasse pith, balsa wood, ground cornstalks, popped corn and like materials.

An object of this invention is a further improvement in explosive compositions. A particular object is to provide a low density dynamite containing as an element of the composition a combustible ingredient of an improved character. A further object of our invention is a low density dynamite having improved sensitiveness properties and one in which the combustible material has relatively low absorbent properties for liquid explosive ingredients, such for example as nitroglycerin. A further object of our invention is an explosive product containing as an ingredient a flaked cereal product. Other and further objects will suggest themselves as our invention is more fully described hereinafter.

Our invention comprises broadly the use in commercial explosives, for example dynamite, of a class of cereal products not heretofore used in explosives and which have been so treated as to be converted into the form of low density flakes. Cereals and cereal products, such as corn, wheat, rye, starch, hominy grits, etc., can be converted into low density flakes by various processes. The one most commonly used and the one which will be described in detail hereinafter is known as the "dry process of milling", as distinguished from the preparation of starch which involves what is known as the "wet process".

In the dry process of milling as applied gen-

erally to maize the hulls and germs are removed and the grains broken into pieces, cooked by steam or other suitable means and pressed to form flakes. This dry process is accomplished by first "tempering" the grains which consists in softening them by means of a small amount of water, this treatment requiring usually from 3 to 4 hours. At the end of the soaking period live steam is injected into the material. The product is then passed to a "degerminator" which breaks up the grain, releasing the germ, the hull, and the softer portion of the starch which surrounds the germ. In this degenerating process the horny portion of the maize kernel is usually cracked or broken into several pieces. It is this horny portion that is most suitable for producing low density flakes. Other starchy portions of course may be flaked by themselves or in combination with the horny portion properly reduced to uniform size. The germ of the cereal grain contains a substantial amount of oil and for this reason it is desirable to remove this from the horny material before flaking.

The resulting material, which at this point may be termed "crude hominy", is then subjected to a cooking process which is intended primarily to slightly soften and preheat the grain before entering the next step in the process. In this cooking process the temperature of the crude hominy is usually raised to approximately 200 to 250° F. The hot, moist material is then subjected to high pressure, for example, by passing through heavy rolls. These rolls operate at a relatively high temperature and the thus treated grains in passing through the rolls are converted into a stiff cohesive flake or sheet.

If the product from the hot rolls is in the form of flakes or sheets then in order to convert these flakes or sheets into proper form for our purpose it is necessary to subject them to a rough grinding process in order to reduce the flakes or sheets to smaller particles suitable for mixing with other explosive ingredients. Flakes of a size suitable for direct use in explosives can be produced provided the grain particles known as grits are sufficiently small in size. We have found that a suitable material is a size that a major portion will pass a 6-mesh screen and at the same time be held on a 60-mesh screen.

There are many variations in the process described in the foregoing, both in the preliminary preparation of the grain and in the handling of the material from the rolls. The essential features of the process however lie in passing a treated cereal or cereal product through hot rolls

in order to convert it into flakes. There are other processes for producing flaked cereal products. For example, another type of process comprises delivering the moist cereal product to a hot roll 5 provided with a scraper where the product is dried and gelatinized and removed from the drum by the scraper. Such processes are well known in the art.

It will be seen at once that this material differs 10 substantially from popped corn covered by Johnson and Baker U. S. Patent 1,687,023, and from the puffed cereal grains covered by the copending application of H. A. Lewis and C. A. Woodbury, Serial No. 602,809, filed April 2, 1932. In 15 both of the latter cases the cereals are not formed into flakes but are exploded or puffed by expansion of vapors locked within the grain.

We have found that the resulting material 20 from processes described in the foregoing has a density between 0.1 and 0.2, this being varied by the method of treatment. We have also found that explosive compositions containing this material as an ingredient have greatly improved properties over similar compositions notwithstanding the fact that some other ingredients 25 have equally low density. The treated or flaked cereal products according to this invention exhibit the unique property of producing low density nitroglycerin explosives of greatly improved sensitiveness or propagating power as 30 compared with similar explosives but containing other low density carbonaceous material such for example as bagasse pith, balsa wood, etc. This cereal product is of particular value in the case 35 of permissible dynamites which at best are noted too sensitive to detonation and of which the lowering of the density by the use of the usual low density absorbents is accompanied by a serious loss in sensitiveness. We have found furthermore 40 that this improved sensitiveness is due to the fact that the combustible material, while low in density, does not readily absorb nitroglycerin or other liquid explosive ingredients that may be present in the composition.

Our invention is applicable to all non-gelatinous types of dynamite compositions, of which the three main classes are commonly known as straight dynamites, ammonia dynamites, and permissible dynamites. The straight dynamites 50 are made in strengths varying from about 20% to 75% and are used in blasting work where high velocity and sensitiveness to detonation are essential. Ordinarily they comprise a liquid explosive ingredient in a percentage equal to their grade strength, combustible absorbents and sodium nitrate. The ammonia dynamites are likewise made in several strengths and are used in general blasting work. They comprise a lower percentage of liquid explosive than the straight 55 dynamites of similar grade, ammonium nitrate, sodium nitrate and combustible absorbents. The 20% ammonia dynamite, for example, may contain 10 to 15% of liquid explosive and 8 to 15% ammonium nitrate, while the 60% ammonia dynamite may have 15 to 30% of liquid explosive 60 and 45 to 60% ammonium nitrate. The permissible dynamites are ordinarily of high grade strength, from 40 to 70%, and are intended for use in coal mines where there is danger of explosion from mine gases and coal dust. These 65 permissible dynamites contain relatively low percentages of liquid explosive, usually between 8 and 15%, and relatively high percentages of ammonium nitrate, 50 to 80%, combustible absorbents, and, in many cases, inorganic salts for the 70 75

purpose of reducing the flame temperature, sodium chloride or sodium nitrate, for example.

While our invention is applicable to many different forms of explosives, the following examples are given to illustrate its applicability to each of the types of dynamite compositions described in the foregoing:

| Ingredient          | Percent. | Percent. | Percent. |
|---------------------|----------|----------|----------|
| Nitroglycerin       | 60       | 23       | 10       |
| Ammonium nitrate    | 32       | 52       | 75       |
| Sodium nitrate      | 20       | 14       | 5        |
| Flaked corn product | 5        | 2        | 5        |
| Other combustible   | 15       | 9        | 2        |

80

85

90

95

100

105

110

115

120

125

130

135

140

145

150

In addition to the improvement in other properties, the low density effect of the use of our new combustible ingredients is shown by the fact that it makes possible the production of straight and ammonia dynamites on otherwise standard formulas, weighing less than 181 grams per 1 1/4 x 8" cartridge, against a weight of 210 to 220 grams ordinarily obtained. Similarly with dynamites of the permissible type, our new ingredient makes it possible to obtain weights of 1 1/4 x 8" cartridges of less than 146 grams, much lower densities being possible with complete utilization of the treated and expanded corn product described in the foregoing.

Various amounts of our improved ingredients 105 may be used in dynamite compositions with satisfactory results. It will be apparent from the foregoing that the higher the percentages we use, replacing the heavier ingredients, the lower will be the density of the finished explosive. While amounts greater than 20 per cent. may be used, the higher percentages have the disadvantage of adding too much carbonaceous combustibles to the explosive. We find also that amounts less than one per cent. are insufficient to have any 115 appreciable effect on either the density or the sensitiveness of the explosive. Preferably we use between 2 and 12 per cent. of our flaked maize product. The use of at least 5 per cent. of liquid explosive ingredient is desirable in our new explosive composition, in the absence of other explosive sensitizers, since a smaller amount than this results in an explosive insufficiently sensitive for satisfactory use.

It will be understood, of course, that the percentages of ingredients given in the foregoing examples may be varied within wide limits, and that additional ingredients may be introduced without departure from the spirit of the invention. Our invention therefore contemplates the 120 use of these low density ingredients as the sole combustible material, or in combination with other combustible ingredients. The other combustible ingredients may be either high density or low density ingredients. For example, it is contemplated that our new explosive may have incorporated therein other low density ingredients such as bagasse pith, balsa wood, popped corn, etc. We may use also in place of nitroglycerin for example, solutions in nitroglycerin of various 125 materials commonly considered as freezing point depressants, nitroglycol, nitrated polymerized glycerin, nitrated sugars, nitrocompounds, etc. The amount of sodium nitrate may likewise be increased or decreased as desired, or omitted entirely, in which case sodium chloride or other flame suppressing material may be used.

Accordingly, it is to be understood that we are to be limited in our invention only as indicated in the following patent claims.

## We claim:

1. A dynamite composition which comprises a liquid explosive ingredient and a flaked cereal product.
- 5 2. A dynamite composition which comprises a liquid explosive ingredient and a degermed flaked cereal product.
3. A dynamite composition which comprises a liquid explosive ingredient and a flaked cereal product having a density between 0.1 and 0.2.
- 10 4. A dynamite composition which comprises a liquid explosive ingredient, and a carbonaceous combustible material comprising a flaked maize product from which the germ and hull portions have been removed.
- 15 5. A dynamite composition which comprises a degermed flaked cereal product and at least 5% of a liquid explosive ingredient.
6. A dynamite composition which comprises a liquid explosive ingredient and 1% to 20% of a flaked cereal product.
- 20 7. An explosive composition of the permissible type characterized by its low density which comprises a liquid explosive ingredient, an inorganic nitrate, a non-explosive salt adapted to reduce flame temperature, and a flaked maize product.
- 25 8. An explosive composition of the ammonium nitrate permissible type containing as an ingredient a flaked maize product, said composition
- having a density such that a 1 $\frac{1}{4}$ " x 8" cartridge weighs less than 146 grams.
9. An explosive composition of the straight dynamite type comprising a liquid explosive ingredient and containing a flaked maize product, said composition having a density such that a 1 $\frac{1}{4}$ " x 8" cartridge weighs less than 181 grams.
10. An explosive composition of the ammonia type comprising a liquid explosive ingredient, ammonium nitrate, and a flaked maize product, said composition having a density such that a 1 $\frac{1}{4}$ " x 8" cartridge weighs less than 181 grams.
11. A low density explosive composition comprising a liquid explosive ingredient, and gelatinized corn flakes.
12. A low density explosive composition comprising a liquid explosive ingredient, and gelatinized cereal flakes cut to desired size.
13. A low density explosive composition comprising a liquid explosive ingredient, ammonium nitrate, a non-explosive salt for reducing the flame temperature, and gelatinized cereal flakes.
14. A low density explosive composition of the permissible type comprising a liquid explosive ingredient, ammonium nitrate, sodium nitrate, and gelatinized corn flakes.

KARL T. GENT.  
NORMAN G. JOHNSON.

30

105

35

110

40

115

45

120

50

125

55

130

60

135

65

140

70

145

75

150